

## 1

3,116,126

## ANTIKNOCK GASOLINE

Wallace L. Richardson, Lafayette, Calif., assignor to California Research Corporation, San Francisco, Calif., a corporation of Delaware  
No Drawing. Filed Sept. 30, 1960, Ser. No. 59,517  
3 Claims. (Cl. 44-69)

This invention relates to a novel antiknock gasoline. More particularly, the invention is concerned with an improved gasoline containing as an antiknock agent a class of superior new lead selenide compounds.

Gasoline compositions of high octane number are commonly required for modern spark ignition internal combustion automobile and aircraft engines. Engines of these types in general use today are designed with high compression ratios for more efficient operation. Since the present trend is toward engines of still higher compression ratios for increased power and improved performance, there is a constant demand for gasoline compositions of even higher octane number.

Improved methods of refining and blending gasoline base stocks, and additives such as lead tetraethyl, have been employed to meet the demands for higher octane number gasoline compositions. However, it has been generally realized that there is at present a limit to the improvement in octane number that can be obtained by such conventional methods and additives. New gasoline base stocks with the combination of different additives are greatly needed, therefore, to avoid present limitations and provide gasoline compositions of high octane number for future use in automobile and aircraft engines.

It has now been found that a superior new gasoline composition of high octane number is provided by a hydrocarbon base fuel boiling in the gasoline boiling range, containing trialkyl lead selenide, preferably, trimethyl lead methyl selenide or trimethyl lead phenyl selenide, a novel and more effective class of lead compounds, in amounts sufficient to improve the octane number, preferably, at least 0.5 milliliter per gallon of base fuel.

The improved gasoline compositions containing the new antiknock compound of the invention show unexpectedly high octane numbers compared to previously known combinations of hydrocarbon base fuels and additives. Hydrocarbon base fuels, together with trialkyl lead selenides and mixtures thereof in accordance with the invention, have octane numbers which are higher than similar base fuels employing the conventional lead tetraethyl additive in the same lead content. This is surprising since it has been generally accepted heretofore that other lead compounds are distinctly less efficient than lead tetraethyl with respect to octane number improvement.

The hydrocarbon base fuel of the composition, according to the invention, is prepared by conventional refining and blending processes. It normally contains straight-chain paraffins, branched-chain paraffins, olefins, aromatics and naphthenes. Since straight-chain paraffins have a tendency to adversely affect octane number, the content of such hydrocarbons is ordinarily low.

As already mentioned, the base fuel is a hydrocarbon fuel boiling in the gasoline boiling range. Generally described, such fuels have an ASTM (D-86) distillation with an initial boiling point of about 100° F. and a final boiling point of about 425° F. Preferably, the unleaded base fuel has a Research octane number of at least 85 as determined by the accepted CFR engine test method. Also, the base fuel preferably contains at least 20 percent by volume of aromatic hydrocarbons. Less than 30 percent by volume of olefinic hydrocarbons are present in the fuel. The total paraffin and naphthene hydrocarbon

## 2

content of the preferred fuel may be as much as 80 percent by volume. For best over-all engine performance, fuels containing in the range of 20 to 60 percent by volume of paraffinic and naphthenic hydrocarbons are preferred for volatility and other desirable gasoline characteristics.

The more preferred hydrocarbon base fuels are also those which contain from 20 to 60 percent by volume aromatic hydrocarbons and from 0 to 30 percent by volume of olefinic hydrocarbons. Most preferably, a gasoline having all-around desirable characteristics has a clear octane number of at least 95 and contains about 50 to 60 percent by volume of paraffin and naphthene hydrocarbons, about 30 to 40 percent aromatic hydrocarbons and about 5 to 15 percent olefinic hydrocarbons.

The trialkyl lead selenides are illustrated by the general formula



in which the  $R_1$ 's are alkyl groups and  $R_2$  is a hydrocarbon radical. The trialkyl lead selenides preferably contain from one to three carbon atoms in each of the alkyl groups attached directly to the lead. The alkyl groups may be the same or different from one another. Particularly preferred for antiknock performance are the trimethyl lead methyl or phenyl selenides.

For practical purposes, not more than about 4 milliliters of lead compounds per gallon is ordinarily used in the compositions. If desired, other octane-improving additives may be employed in addition to trialkyl lead selenide. These include other lead compounds such as lead tetraethyl, carbonyl derivatives of iron and cyclopentadienyl derivatives of metals such as manganese or iron. Other gasoline additives, such as scavengers like ethylene chloride or bromide, oxidation inhibitors, corrosion inhibitors, surface ignition suppressants like phosphorus compounds, detergents, and the like may be present.

The following examples illustrate the preparation of trialkyl lead selenide compounds in accordance with this invention. Unless otherwise specified the proportions are on a weight basis.

## EXAMPLE I

This example shows the preparation of trimethyl lead methyl selenide. One-half mole of methyl magnesium bromide is treated with one-half mole of powdered selenium. The resulting intermediate methyl selenomagnesium bromide is treated directly with one-half mole of trimethyl lead chloride. A mildly exothermic reaction occurs, and the mixture is rapidly stirred and refluxed for one-half hour. An ice-cold solution of ammonium chloride is added to remove the magnesium salts, and the seleno-lead compound is extracted with ethyl ether. The extract is dried and the ether is removed in vacuo at room temperature. The isolated product is a yellow oil obtained in a yield of 50 percent based on selenium. The boiling point is 75° C. at a pressure of 3 mm. of mercury and the compound boils with slight decomposition. The specific gravity at 20° C. is 2.42.

## EXAMPLE II

This example shows the preparation of trimethyl lead phenyl selenide. A solution of 0.2 mole of phenyl magnesium bromide in 300 ml. anhydrous ethyl ether is treated with 15 g. (0.18 mole) of finely powdered selenium. A vigorous reaction follows this addition, and the reaction is completed by refluxing the material for one-half hour. Sixty-three grams (0.18 mole) of trimethyl lead chloride is added gradually. A very mild exothermic reaction occurs, and the mixture becomes dark

brown. The materials are refluxed for 1½ hours. The magnesium salts are removed by treatment with an ice-cold solution of ammonium chloride, and the product is extracted with ethyl ether, dried over anhydrous magnesium sulfate, and the ether is removed under vacuum. The product is isolated as an orange-colored oil having a specific gravity of 2.60. The yield based on the selenium is 60 percent.

In further illustration of the superior new gasoline antiknock compound of the invention, several compositions and tests thereon are given in the following examples. These tests show the improved effect of the combination of the particular hydrocarbon base fuel with trialkyl lead selenide compounds as compared with fuels containing other lead compounds.

The following table is a summary of the pertinent data of the examples. The hydrocarbon base fuel has a Research octane of 94.4 and contains 51 percent by volume of the paraffins and naphthenes, 25 percent olefins, and 24 percent aromatics. The table shows the effect on octane number by the addition of representative trialkyl lead selenides, as compared to lead tetraethyl. The octane numbers in this comparison are based on the Research Method D-908 and the Motor Method D-357 of the "ASTM Manual of Engine Test Methods for Rating Fuels." The latter method, which is more stringent than the Research Method, illustrates more accurately the desirable qualities of the improved gasoline composition of the invention.

In the table, the effect of trialkyl lead selenide compared with lead tetraethyl is based on gasoline compositions containing an equal lead concentration. For the purpose of practical comparison this is 3.17 grams of lead per gallon. Such amounts are equivalent to the 3 cc. of tetraethyl lead per gallon employed in many gases. The "Improvement" is the difference in the octane number obtained with trimethyl lead selenide compound less the octane number obtained with the equivalent amount of lead tetraethyl.

Table

| Example No. | Lead Compound                  | Research Octane | Improvement | Motor Octane | Improvement |
|-------------|--------------------------------|-----------------|-------------|--------------|-------------|
| III-----    | Tetraethyl Lead                | 99.2            |             | 87.7         |             |
| IV-----     | Trimethyl lead phenyl selenide | 99.4            | +0.2        | 88.2         | +0.5        |
| V-----      | Trimethyl lead methyl selenide | 99.5            | +0.3        | 88.0         | +0.3        |

The examples summarized in the above table show that the improved gasoline composition of the invention containing trialkyl lead selenide is surprisingly better on the basis of octane number rating than comparable gasoline compositions of the type known heretofore.

The organolead compounds of this invention are also useful wherever oil-soluble lead compounds are desired. For example, fine particle dispersions of lead may be obtained by thermal decomposition of the trialkyl lead selenide dissolved in liquid hydrocarbon, such as isoocane. Such fine metal dispersions of lead are useful as

catalysts for certain reactions. The fine lead particles may be converted to lead oxides which are useful as lubrication agents. The lead compound of the invention may also be used as a free radical initiator in polymerization reactions.

I claim:

1. A hydrocarbon fuel of the gasoline boiling range adapted for use as a fuel for spark ignition internal combustion engines containing at least 20 percent by volume of aromatic hydrocarbons, less than 30 percent by volume of olefinic hydrocarbons and not more than 80 percent by volume of paraffinic and naphthenic hydrocarbons, said hydrocarbon fuel having incorporated therein an amount sufficient to improve the octane number of trialkyl lead selenide of the formula



20 in which  $\text{R}_1$  is methyl and  $\text{R}_2$  is selected from the group consisting of methyl and phenyl.

2. A hydrocarbon base fuel of the gasoline boiling range having an octane number of at least 85 and containing at least 20 percent by volume of aromatic hydrocarbons, less than 30 percent by volume of olefinic hydrocarbons and not more than 80 percent by volume of paraffinic and naphthenic hydrocarbons, said hydrocarbon fuel having incorporated therein trimethyl lead phenyl selenide in an amount sufficient to improve the octane number.

3. A hydrocarbon base fuel of the gasoline boiling range having an octane number of at least 85 and containing at least 20 percent by volume of aromatic hydrocarbons, less than 30 percent by volume of olefinic hydrocarbons and not more than 80 percent by volume of paraffinic and naphthenic hydrocarbons, said hydrocarbon fuel having incorporated therein trimethyl lead methyl selenide in an amount sufficient to improve the octane number.

40

## References Cited in the file of this patent

## UNITED STATES PATENTS

|           |                  |                |
|-----------|------------------|----------------|
| 1,592,955 | Midgley          | July 20, 1926  |
| 1,601,215 | Johansen         | Sept. 28, 1926 |
| 1,635,216 | Kettering et al. | July 12, 1927  |
| 2,150,349 | Van Peski et al. | Mar. 14, 1939  |
| 2,314,575 | Doran            | Mar. 23, 1943  |
| 2,375,236 | Miller           | May 8, 1945    |
| 2,447,926 | Wiczer           | Aug. 24, 1948  |
| 2,893,857 | De Pree          | July 7, 1959   |

## FOREIGN PATENTS

|         |               |               |
|---------|---------------|---------------|
| 448,620 | Germany       | Aug. 24, 1927 |
| 267,079 | Great Britain | Nov. 24, 1927 |

## OTHER REFERENCES

"Improved Motor Fuels Through Selective Blending," by Wagner, paper presented before 22nd Annual Meeting to the American Petroleum Institute, Nov. 7, 1941, 60 pp. 8-13.